



SPECTRALLY SENSITIZED SILVER HALIDE  
PHOTOGRAPHIC MATERIAL

BACKGROUND OF THE INVENTION

This invention relates to a spectrally sensitized silver halide photographic material, more particularly to a silver halide photographic material that is low in fog, that has enhanced spectral sensitivity and that can be stored for a prolonged time without deterioration after its preparation (i.e. has good raw stock stability).

As is well known, certain kinds of cyanine dyes and merocyanine dyes are very effective means of spectrally sensitizing silver halide emulsions. However, these dyes, if used alone, are incapable of providing sufficient sensitivity and they are usually combined with certain other spectral sensitizers or organic compounds to attain higher sensitivity by providing emulsions with sensitivity that is greater than the simple sum of the sensitivities achievable by the individual compounds. This effect is commonly known in the art as "supersensitization".

Generally speaking, the addition of a second dye or organic material will often either fail to increase the sensitivity or reduce it, so supersensitization may well be regarded as a peculiar phenomenon and the organic compound or second sensitizing dye to be combined must be selected with extremely close tolerance. Thus, a seemingly slight difference in chemical structure can cause marked effects on the supersensitizing action and it is difficult to obtain an appropriate combination for supersensitization merely by prediction from chemical structural formulas.

When spectral sensitizers are to be used to achieve supersensitization in silver halide photographic emulsions, they are required to provide high spectral sensitivity. It is well known that styryl bases exhibit a strong supersensitizing action in the spectral sensitization of silver halides with monomethine cyanine dyes. See, for example, T. H. James, "The Theory of the Photographic Process", Fourth Edition, p. 264, Macmillan Publishing Co., Inc., New York, 1977.

It is also known that styryl bases exhibit a strong 45 supersensitizing action in the spectral sensitization of silver halides with various other cyanine dyes (see, for example, U.S. Pat. No. 2,313,922).

In both references mentioned above, the styryl bases used are those represented by the following general 50 formula (IV) having an amino group on the benzene ring which is substituted by a substituted or unsubstituted alkyl group:



where Z is the nonmetallic atomic group necessary to form a 5- or 6-membered hetero ring; r is 0 or 1; and R is a substituted or unsubstituted alkyl group. However, silver halide photographic emulsions supersensitized by these methods are still unsatisfactory in terms of spectral sensitivity; further, they are prone to suffer from increased fog and the raw stock stability of light-sensitive samples is also insufficient.

SUMMARY OF THE INVENTION

An object, therefore, of the present invention is to provide a silver halide photographic material that is low in fog, that has enhanced spectral sensitivity and that can be stored for a prolonged time without deterioration after its preparation.

The present inventors conducted intensive studies in order to develop a silver halide photographic material that satisfies their need and found that the above-stated object of the present invention can be attained by a silver halide photographic material having one or more light-sensitive silver halide emulsion layers on a support, which photographic material is characterized in that at least one of said light-sensitive emulsion layers contains silver halide grains that are spectrally sensitized with at least one of the spectral sensitizers represented by the following general formula (I) and further contains at least one of the compounds represented by the following general formulas (II) and (III):

(I)



where  $Z_1$  and  $Z_2$  each represents the atomic group necessary to form a 5- or 6-membered nitrogenous hetero ring;  $L_1$ ,  $L_2$ ,  $L_3$ ,  $L_4$  and  $L_5$  are each a methine group;  $R_1$  and  $R_2$  are each independently a substituted or unsubstituted alkyl group;  $X_1$  is a charge balancing counter ion;  $K_1$  represents a value of zero or more for neutralizing electric charges;  $k_1$  and  $k_2$  are each an integer of 0 or 1; and  $m$  and  $n$  are each an integer of 0-2;



where  $Z_3$  is an oxygen atom, a sulfur atom, a selenium atom, a tellurium atom or



group;  $V_{21}$ ,  $V_{22}$ ,  $V_{23}$  and  $V_{24}$  are each a hydrogen atom, a halogen atom, an aryl group, an alkyl group, a substituted alkyl group, an alkoxy group, an alkoxy carbonyl group, a carboxyl group, a hydroxyl group or a cyano group, provided that  $V_{21}$  and  $V_{22}$ , or  $V_{22}$  and  $V_{23}$  or  $V_{23}$  and  $V_{24}$  may be condensed together to form a benzene ring;  $R_{21}$ ,  $R_{22}$ ,  $R_{23}$ ,  $R_{24}$  and  $R_{25}$  are each a hydrogen atom, a halogen atom, a hydroxyl group, an alkyl group, an alkoxy group, an aryl group or a group capable of forming a 5- or 6-membered ring through condensation of adjacent substituents; and  $R_{26}$  is a substituted or unsubstituted alkyl or aryl group;



(III)

where  $Z_4$  has the same meaning as  $Z_3$ ;  $V_{31}$ ,  $V_{32}$ ,  $V_{33}$  and  $V_{34}$  have the same meanings as  $V_{21}$ ,  $V_{22}$ ,  $V_{23}$  and  $V_{24}$ ;  $R_{31}$ ,  $R_{32}$ ,  $R_{33}$ ,  $R_{34}$  and  $R_{35}$  have the same meanings as  $R_{21}$ ,  $R_{22}$ ,  $R_{23}$ ,  $R_{24}$  and  $R_{25}$ ;  $X_2$  and  $K_2$  have the same meanings as  $X_1$  and  $K_1$ ; and  $R_{36}$  is substituted or unsubstituted alkyl or aryl group.

The objects of the present invention can be accomplished more effectively if the silver halide grains contained in at least one light-sensitive silver halide emulsion layer which are spectrally sensitized with at least one of the spectral sensitizers of the general formula (I) have a core/shell structure.

#### DETAILED DESCRIPTION OF THE INVENTION

The general formula (I) is described below in detail.

The nitrogenous hetero rings formed by  $Z_1$  and  $Z_2$  in the general formula (I) are 5- or 6-membered hetero rings commonly used in cyanine dyes, or those rings which are formed by condensing said 5- or 6-membered hetero rings with a benzene or naphthalene ring. Examples of the hetero rings formed by  $Z_1$  and  $Z_2$  are cyanine heterocyclic nuclei that are composed of a thiazole ring, a selenazole ring, an oxazole ring, a tetrazole ring, a pyridine ring, a pyrrolidine ring or an imidazole ring and which have substituents on the ring.

More specific examples include: thiazolic nuclei such as thiazole, 4-methylthiazole, 4-phenylthiazole, 5-methylthiazole, 5-phenylthiazole, 4,5-dimethylthiazole, 4,5-diphenylthiazole, benzothiazole, 5-fluorobenzothiazole, 5-chlorobenzothiazole, 6-chlorobenzothiazole, 5-methylbenzothiazole, 6-methylbenzothiazole, 5-bromobenzothiazole, 5-carboxybenzothiazole, 5-ethoxybenzothiazole, 5-hydroxybenzothiazole, 5-phenylbenzothiazole, 6-phenylbenzothiazole, 5-methoxybenzothiazole, 6-methoxybenzothiazole, 5-iodobenzothiazole, 6-ethoxybenzothiazole, tetrahydrobenzothiazole, 5,6-dimethylbenzothiazole, 5,6-dimethoxybenzothiazole, 5,6-dioxymethylenebenzothiazole, 6-ethoxy-5-methylbenzothiazole, 5-phenethylbenzothiazole, naphtho[1,2-d]thiazole, naphtho[2,1-d]thiazole, naphtho[2,3-d]thiazole, 5-methoxynaphtho[1,2-d]thiazole, 5-methoxynaphtho[2,1-d]thiazole, 8-methoxynaphtho[2,1-d]thiazole, 7-methoxynaphtho[2,1-d]thiazole, 5-methoxythionaphtheno[6,7-d]thiazole, 5-methoxythionaphtheno[6,7-d]-8,9-dihydroneaphtho[1,2-d]thiazole and 4,5-dihydroneaphtho[2,1-d]thiazole; oxazolic nuclei such as 4-methyloxazole, 5-methyloxazole, 4-phenyloxazole, 4,5-dimethyloxazole, 5-phenyloxazole, 5,6-diphenyloxazole, benzoxazole, 5-chlorobenzoxazole, 5-methylbenzoxazole, 5-phenylbenzoxazole, 6-methylbenzoxazole, 5,6-dimethylbenzoxazole, 5-methoxybenzoxazole, 5-hydroxybenzoxazole, ethoxycarbonylbenzoxazole, 5-bromobenzoxazole, 5-methyl-6-chlorobenzoxazole, naphtho[1,2-d]oxazole, naphtho[2,1-d]oxazole and naphtho[2,3-d]oxazole; selenazolic nuclei such as 4-methylselenazole, 4-phenylselenazole, benzoselenazole,

10

15

20

25

30

35

40

45

50

55

60

65

chlorobenzoselenazole, 5-methoxybenzoselenazole, 5-methylbenzoselenazole, tetrahydrobenzoselenazole, naphtho[1,2-d]selenazole, and naphtho[2,1-d]selenazole; tetrazolic nuclei such as 4-phenyltetrazole, 4-methyltetrazole, benzotetrazole, 5-methoxybenzotetrazole, 5,6-dimethylbenzotetrazole, naphtho[2,1-d]tetrazole and naphtho[1,2-d]tetrazole; pyridinic nuclei such as 2-pyridine, 5-methyl-2-pyridine, 4-pyridine and 3-methyl-4-pyridine; quinolinic nuclei such as 2-quinoline, 6-methyl-2-quinoline, 5-ethyl-2-quinoline, 6-chloro-2-quinoline, 8-chloro-2-quinoline, 6-methoxy-2-quinoline, 8-ethoxy-2-quinoline, 6-methyl-2-quinoline, 8-fluoro-2-quinoline, 6-dimethylamino-2-quinoline, 4-quinoline, 6-methoxy-4-quinoline, 7-methyl-4-quinoline, and 8-chloro-4-quinoline; 3,3-dialkylindolenic nuclei such as 3,3-dimethylindoline, 3,3,5-trimethylindoline, 3,3-dimethyl-5-(dimethylamino)indoline and 3,3-diethylindoline; imidazolic nuclei such as imidazole, 1-alkylimidazole, 1-alkyl-4-phenylimidazole, 1-alkyl-4,5-dimethylimidazole, 1-alkylbenzimidazole, 1-phenyl-5,6-dichlorobenzimidazole, 1-alkyl-5-cyanobenzimidazole, 1-alkyl-5-chlorobenzimidazole, 1-alkyl-5,6-dichlorobenzimidazole, 1-alkyl-5-chloro-6-cyanobenzimidazole, 1-alkyl-5-trifluoromethylbenzimidazole, 1-alkyl-5-methylsulfonylbenzimidazole, 1-alkyl-5-methoxycarbonylbenzimidazole, 1-alkyl-5-acetylbenzimidazole, 1-alkyl-5-(N,N-dimethylamino)sulfonylbenzimidazole, 1-alkylnaphtho[1,2-d]imidazole, 1-alkylnaphtho[2,1-d]imidazole and 1-alkylnaphtho[2,3-d]imidazole.

The 1-alkyl groups mentioned above are alkyl groups having 1-10 carbon atoms, exclusive of the carbon atoms in substituents if they are present. Also included in the category of 1-alkyl groups are those which are substituted by alkoxy groups of  $C_{1-6}$ , alkoxy carbonyl groups having alkoxy groups of  $C_{1-4}$ , a carboxyl group, a carbamoyl group, a cyano group, a halogen atom, a sulfo atom, a phenyl group, a substituted phenyl group or a vinyl group. Specific examples of substituents include methyl, ethyl, cyclohexyl, butyl, decyl, 2-methoxyethyl, 3-butoxypropyl, 2-hydroxy-ethoxyethyl, ethoxycarbonylmethyl, carboxymethyl, 2-carboxyethyl, 2-cyanoethyl, 2-carbamoylethyl, 2-hydroxyethyl, 2-fluoroethyl, 2,2,2-trifluoroethyl, 2-sulfoethyl, 3-sulfo-propyl, 4-sulfobutyl, phenethyl, benzyl, sulfophenethyl, carboxybenzyl, allyl, etc.

The nuclei formed by  $Z_1$  and  $Z_2$  may further exemplified by the following: oxazolinic nuclei such as oxazoline and 4,4-dimethyloxazoline; thiazolinic nuclei such as thiazoline and 4-methylthiazoline; isoxazolic nuclei such as isoxazole, benzisoxazole, 5-chlorobenzisoxazole, 6-methylbenzisoxazole, 7-methylbenzoxazole, 6-methoxybenzoxazole and 7-methoxybenzisoxazole; 1,3,4-thiadiazolic nuclei such as 5-methyl-1,3,4-thiadiazole and 5-methylthio-1,3,4-thiadiazole; thiethiothiazolic nuclei such as thieno[2,3-d]thiazole, thieno[3,2-d]thiazole, thieno[2,3-e]benzothiazole, thieno[3,2-e]benzothiazole and thiazolo[4,5-b]benzothiophene; tetrazolic nuclei such as 1-alkyltetrazole; imidazoquinolinic nuclei such as 1-alkylimidazo[4,5-b]quinoxaline, 6,7-dichloro-1-alkylimidazo[4,5-b]quinoxaline and 6-dichloro-1-allylimidazo[4,5-b]quinoxaline; imidazoquinolinic nuclei such as 1-alkylimidazo[4,5-b]quinoline and 6,7-dichloro-1-alkylimidazo[4,5-b]quinoline; pyrrolopyridinic nuclei such as 3,3-dialkyl-3H-pyrrolo[2,3-b]pyridine; pyr-

rolopyrazinic nuclei such as pyrrolo[2,3-b]pyrazine; and pyridopyridinic nuclei such as pyrido[2,3-b]pyridine.

The methine groups represented by L<sub>1</sub>-L<sub>5</sub> may have substituents exemplified by the following: lower alkyl groups having 1-6 carbon atoms such as methyl, ethyl, propyl and isopropyl; aryl groups such as phenyl, p-tolyl and p-chlorophenyl; alkoxy groups having 1-4 carbon atoms such as methoxy and ethoxy; aryloxy groups such as phenoxy; aralkyl groups such as benzyl and phenethyl; heterocyclic groups such as thienyl and furyl; substituted amino groups such as dimethylamino, tetramethyleneamino and anilino; alkylthio groups such as methylthio; and acidic nucleus containing groups such as malononitrile, alkylsulfonylacetonitrile, cyanomethylbenzofuranylketone or cyanomethylphenylketone, 2-pyrazolin-5-one, pyrazolidin-3,5-dione, imidazolin-5-one, hydantoin, 2- or 4-thiohydantoin, 2-iminooxazolin-4-one, 2-oxazolin-5-one, 2-thioxazolidine, 2,4-dione, isoxazolin-5-one, 2-thiazolin-4-one, thiazolidin-4-one, thiazolidine-2,4-dione, rhodanine, thiazolidine-2,4-dithione, isorhodanine, indane-1,3-dione, thiophen-3-one, thiophene-3,1,1-dioxide, indolin-2-one, indolin-3-one, indazolin-3-one, 2-oxoimidazolinium, 3-oxoindazolinium, 5,7-dioxo-6,7-dihydrothiazolo[3,2-a]pyrimidine, cyclohexane-1,3-dione, 3,4-dihydroisoquinolin-4-one, 1,3-dioxane-4,6-dione, barbituric acid, 2-thiobarbituric acid, chroman-2,4-dione, indazolin-2-one and pyrido[1,2-a]pyrimidine-1,3-dione. If desired, substituents on the methine chain may combine together to form 4- to 6-membered rings such as a 2-hydroxy-4-oxocyclobutene ring, a cyclopentane ring and a 3,3-dimethylcyclohexene ring.

The alkyl groups represented by R<sub>1</sub> and R<sub>2</sub> are preferably those having 1-8 carbon atoms, such as methyl, ethyl, butyl and isobutyl. Such alkyl groups may have substituents as exemplified by an alkoxy group, an alkoxycarbonyl group, an aryl group, a hydroxy group, a cyano group, a vinyl group, a halogen atom, a carbamoyl group, a sulfamoyl group, a carboxyl group, a sulfo group, a sulfato group, etc.

The symbol (X<sub>1</sub>)K<sub>1</sub> is included within the formula (I) in order to indicate the presence or absence of cations or anions that are necessary to neutralize the ionic charges in the dye. Hence, K<sub>1</sub> may assume any value of 0 or greater as appropriate for a specific need. Whether a given dye is a cation, an anion or is devoid of net ionic charges will depend on the associated auxochrome and the substituents present. Typical cations are inorganic or organic ammonium ions (e.g. triethylammonium ion and pyridinium ion), alkali metal ions (e.g. sodium ion and potassium ion), and alkaline earth metal ions (e.g. calcium ion and strontium ion). Typical anions are specifically exemplified by halide anions (e.g. chloride ion, bromide ion and iodide ion), substituted arylsulfonic acid ions (e.g. p-toluenesulfonic acid ion and p-chlorobenzenesulfonic acid ion), arylsulfonic acid ions (e.g. 1,3-benzenedisulfonic acid ion and 1,5-naphthalenedisulfonic acid ion), alkylsulfuric acid ions (e.g. methylsulfuric acid ion), sulfuric acid ion, thiocyanic acid ion, perchloric acid ion, tetrafluoroboric acid ion, picric acid ion, acetic acid ion, and trifluoromethanesulfonate acid ion.

Among the compounds represented by the general formula (I), compounds that are represented by the following general formulas (Ia) and (Ib) are particularly preferred:



where R<sub>1</sub>, R<sub>2</sub>, X<sub>1</sub> and K<sub>1</sub> have the same meanings as defined in the general formula (I); Y<sub>1</sub> and Y<sub>2</sub> are each an oxygen atom, a sulfur atom, a selenium atom, a tellurium atom or



V<sub>1</sub>-V<sub>8</sub> are each a hydrogen atom, an alkyl group (e.g. methyl, ethyl or trifluoromethyl), an alkoxy group (e.g. methoxy or ethoxy), a halogen atom (e.g. F, Cl or Br), a phenyl group, a hydroxyl group, a cyano group, an alkoxycarbonyl group (e.g. methoxycarbonyl or butoxycarbonyl), a carbamoyl group (e.g. carbamoyl or N,N-dimethylaminocarbonyl), a sulfamoyl group (e.g. sulfamoyl or N,N-pentamethyleneaminosulfonyl), or a sulfonyl group (e.g. methanesulfonyl or benzenesulfonyl); V<sub>1</sub> and V<sub>2</sub>, or V<sub>2</sub> and V<sub>3</sub>, or V<sub>3</sub> and V<sub>4</sub>, or V<sub>5</sub> and V<sub>6</sub>, or V<sub>6</sub> and V<sub>7</sub>, or V<sub>7</sub> and V<sub>8</sub> may combine with each other to form a benzene ring, a cyclohexene ring, a thiophene ring, etc.; R<sub>4</sub> is a substituted or unsubstituted alkyl or aryl group.; W<sub>1</sub>-W<sub>4</sub> are each a hydrogen atom, an alkyl group (e.g. methyl or ethyl) or a phenyl group, provided that in a preferred case W<sub>1</sub> and W<sub>2</sub> and/or W<sub>3</sub> and W<sub>4</sub> may combine with each other to form a benzene ring, a cyclohexene ring, a thiophene ring or a naphthalene ring, with the following substituents being optionally present on these rings: a halogen atom (e.g. F, Cl or Br), an alkyl group (e.g. methyl or ethyl), an alkoxy group (e.g. methoxy or ethoxy), an aryl group (e.g. phenyl), a trifluoromethyl group, a cyano group, an alkoxycarbonyl group (e.g. methoxycarbonyl or butoxycarbonyl), a carbamoyl group (e.g. carbamoyl or N,N-dimethylaminocarbonyl), a sulfonyl group (e.g. methanesulfonyl or benzenesulfonyl), a sulfamoyl group (e.g. sulfamoyl or N,N-dimethylaminosulfonyl), etc.; R<sub>3</sub> is a hydrogen atom, an alkyl group (e.g. methyl, ethyl, propyl or n-butyl), an aralkyl group (e.g. benzyl), an aryl group (e.g. phenyl or p-tolyl), a heterocyclic group (e.g. 2-furyl or 2-thienyl), an acidic nucleus containing group (e.g. 2,4,6-triketohexahydropyrimidine derivative, pyrazolone derivative, 2-thio-2,4,6-triketohexahydropyrimidine derivative, hydantoin derivative, indandione derivative, thianaphthenone derivative; or oxazolone derivative).

Specific but by no means limiting examples of the spectral sensitizers to be used in the present invention that are represented by the general formula (I) are listed below.



| I-No. | V <sub>2</sub>  | V <sub>3</sub>   | V <sub>6</sub>   | V <sub>7</sub> | R <sub>1</sub>                                                                    | R <sub>2</sub>                                               | (X <sub>1</sub> )k <sub>1</sub> |
|-------|-----------------|------------------|------------------|----------------|-----------------------------------------------------------------------------------|--------------------------------------------------------------|---------------------------------|
| 1     | H               | Cl               | Cl               | H              | (CH <sub>2</sub> ) <sub>4</sub> SO <sub>3</sub> <sup>⊖</sup>                      | (CH <sub>2</sub> ) <sub>4</sub> SO <sub>3</sub> Na           | —                               |
| 2     | H               | Cl               | Cl               | H              | (CH <sub>2</sub> ) <sub>4</sub> SO <sub>3</sub> <sup>⊖</sup>                      | CH <sub>2</sub> COOH                                         | —                               |
| 3     | H               | OCH <sub>3</sub> | OCH <sub>3</sub> | H              | (CH <sub>2</sub> ) <sub>3</sub> SO <sub>3</sub> <sup>⊖</sup>                      | (CH <sub>2</sub> ) <sub>3</sub> SO <sub>3</sub> Na           | —                               |
| 4     | H               | H                | H                | H              | (CH <sub>2</sub> )<br> <br>CHCH <sub>3</sub><br> <br>SO <sub>3</sub> <sup>⊖</sup> | CH <sub>2</sub> CH=CH                                        | —                               |
| 5     | H               | OCH <sub>3</sub> | OH               | H              | (CH <sub>2</sub> ) <sub>2</sub> SO <sub>3</sub> <sup>⊖</sup>                      | (CH <sub>2</sub> ) <sub>2</sub> SO <sub>3</sub> Na           | —                               |
| 6     | CH <sub>3</sub> | CH <sub>3</sub>  | Cl               | H              | (CH <sub>2</sub> ) <sub>2</sub> COOH                                              | (CH <sub>2</sub> ) <sub>2</sub> SO <sub>3</sub> <sup>⊖</sup> | —                               |



-continued

I-13



I-14



I-15



I-16



I-17



I-18



I-19



I-20



I-21



-continued

I-22



I-23



I-24



I-25



I-26



I-27



I-28



I-29



I-30



[Ib-1]



| I-No. | V <sub>10</sub> | V <sub>11</sub>                  | V <sub>12</sub>                  | V <sub>13</sub>                 | R <sub>1</sub>                                                                       | R <sub>2</sub>                                                                                   | R <sub>3</sub>                | (X <sub>1</sub> )k <sub>1</sub> |
|-------|-----------------|----------------------------------|----------------------------------|---------------------------------|--------------------------------------------------------------------------------------|--------------------------------------------------------------------------------------------------|-------------------------------|---------------------------------|
| 31    | H               | COCH <sub>3</sub>                | COCH <sub>3</sub>                | H                               | (CH <sub>2</sub> ) <sub>3</sub> SO <sub>3</sub> <sup>⊖</sup>                         | (CH <sub>2</sub> ) <sub>3</sub> SO <sub>3</sub> Na                                               | C <sub>2</sub> H <sub>5</sub> | —                               |
| 32    | H               |                                  |                                  | H                               | (CH <sub>2</sub> ) <sub>4</sub> SO <sub>3</sub> <sup>⊖</sup>                         | (CH <sub>2</sub> ) <sub>4</sub> SO <sub>3</sub> H.N(C <sub>2</sub> H <sub>5</sub> ) <sub>3</sub> | C <sub>2</sub> H <sub>5</sub> | —                               |
| 33    | H               |                                  | Cl                               | H                               | (CH <sub>2</sub> ) <sub>2</sub> CH <sub>2</sub><br> <br>SO <sub>3</sub> <sup>⊖</sup> | (CH <sub>2</sub> ) <sub>3</sub> SO <sub>3</sub> H.N(C <sub>2</sub> H <sub>5</sub> ) <sub>3</sub> | C <sub>2</sub> H <sub>5</sub> | —                               |
| 34    | H               | Cl                               | Cl                               | H                               | (CH <sub>2</sub> ) <sub>3</sub> SO <sub>3</sub> <sup>⊖</sup>                         | (CH <sub>2</sub> ) <sub>3</sub> SO <sub>3</sub> H.N(C <sub>2</sub> H <sub>5</sub> ) <sub>3</sub> | C <sub>2</sub> H <sub>5</sub> | —                               |
| 35    | H               |                                  |                                  | H                               | (CH <sub>2</sub> ) <sub>3</sub> SO <sub>3</sub> <sup>⊖</sup>                         | (CH <sub>2</sub> ) <sub>3</sub> SO <sub>3</sub> H.N<br>                                          | C <sub>2</sub> H <sub>5</sub> | —                               |
| 36    | H               | OCH <sub>3</sub>                 | OCH <sub>3</sub>                 | H                               | (CH <sub>2</sub> ) <sub>3</sub> SO <sub>3</sub> <sup>⊖</sup>                         | C <sub>2</sub> H <sub>5</sub>                                                                    | C <sub>2</sub> H <sub>5</sub> | —                               |
| 37    | H               | COOC <sub>2</sub> H <sub>5</sub> | COOC <sub>2</sub> H <sub>5</sub> | H                               | (CH <sub>2</sub> ) <sub>3</sub> SO <sub>3</sub> <sup>⊖</sup>                         | C <sub>2</sub> H <sub>5</sub>                                                                    | C <sub>2</sub> H <sub>5</sub> | —                               |
| 38    | H               |                                  |                                  | H                               | (CH <sub>2</sub> ) <sub>2</sub> SO <sub>3</sub> <sup>⊖</sup>                         | (CH <sub>2</sub> ) <sub>2</sub> SO <sub>3</sub> Na                                               | C <sub>2</sub> H <sub>5</sub> | —                               |
| 39    | H               | Cl                               | Cl                               | CH <sub>3</sub>                 | (CH <sub>2</sub> ) <sub>3</sub> SO <sub>3</sub> <sup>⊖</sup>                         | (CH <sub>2</sub> ) <sub>4</sub> SO <sub>3</sub> H.N(C <sub>2</sub> H <sub>5</sub> ) <sub>3</sub> | C <sub>2</sub> H <sub>5</sub> | —                               |
| 40    | H               | Cl                               | Cl                               | H                               | (CH <sub>2</sub> ) <sub>3</sub> SO <sub>3</sub> <sup>⊖</sup>                         | (CH <sub>2</sub> ) <sub>3</sub> SO <sub>3</sub> <sup>⊖</sup>                                     | C <sub>2</sub> H <sub>5</sub> | —                               |
| 41    | H               |                                  |                                  | H                               | C <sub>2</sub> H <sub>5</sub>                                                        | C <sub>2</sub> H <sub>5</sub>                                                                    |                               | I <sup>⊖</sup>                  |
| 42    | H               |                                  | t-C <sub>5</sub> H <sub>11</sub> | H                               | (CH <sub>2</sub> ) <sub>2</sub> SO <sub>3</sub> <sup>⊖</sup>                         | (CH <sub>2</sub> ) <sub>4</sub> SO <sub>3</sub> H.N(C <sub>2</sub> H <sub>5</sub> ) <sub>3</sub> | C <sub>2</sub> H <sub>5</sub> | —                               |
| 43    | H               |                                  | CH <sub>2</sub><br>—<br>         | H                               | (CH <sub>2</sub> ) <sub>3</sub> SO <sub>3</sub> <sup>⊖</sup>                         | (CH <sub>2</sub> ) <sub>3</sub> SO <sub>3</sub> Na                                               | C <sub>2</sub> H <sub>5</sub> | —                               |
| 44    | H               |                                  | H                                | t-C <sub>4</sub> H <sub>9</sub> | (CH <sub>2</sub> ) <sub>3</sub> SO <sub>3</sub> <sup>⊖</sup>                         | (CH <sub>2</sub> ) <sub>3</sub> SO <sub>3</sub> K                                                | C <sub>2</sub> H <sub>5</sub> | —                               |
| 45    | H               | F                                | F                                | H                               | (CH <sub>2</sub> ) <sub>2</sub> NH<br> <br>SO <sub>2</sub> CH <sub>3</sub>           | (CH <sub>2</sub> ) <sub>4</sub> SO <sub>3</sub> <sup>⊖</sup>                                     | H                             | —                               |
| 46    | H               |                                  |                                  | H                               | (CH <sub>2</sub> ) <sub>2</sub> SO <sub>3</sub> <sup>⊖</sup>                         | (CH <sub>2</sub> ) <sub>2</sub> SO <sub>3</sub> H.N<br>                                          | H                             | —                               |
| 47    | H               | Br                               | Br                               | H                               | (CH <sub>2</sub> ) <sub>4</sub> SO <sub>3</sub> <sup>⊖</sup>                         | (CH <sub>2</sub> ) <sub>4</sub> SO <sub>3</sub> Na                                               | C <sub>3</sub> H <sub>7</sub> | —                               |

-continued

|    |   |    |   |                  |                             |          |   |
|----|---|----|---|------------------|-----------------------------|----------|---|
| 48 | H | Cl | H | $(CH_2)_2SO_3^-$ | $(CH_2)_3SO_3H.N(C_2H_5)_3$ | $C_2H_5$ | — |
|----|---|----|---|------------------|-----------------------------|----------|---|



-continued

I-57



I-58



I-59



I-60



I-61



I-62



I-63



I-64



I-65



-continued

I-66



I-67



I-68



I-69



I-70



I-71



I-72



I-73



-continued

I-74



I-75



I-76



I-77



I-78



I-79



I-80



I-81



I-82



-continued

I-83



[Ib-2]



| I-No. | V <sub>10</sub>  | V <sub>11</sub>                  | V <sub>12</sub>  | V <sub>13</sub> | R <sub>1</sub>                                               | R <sub>2</sub>                                                                                                                           | R <sub>3</sub>                | (X <sub>1</sub> )k <sub>1</sub> |   |
|-------|------------------|----------------------------------|------------------|-----------------|--------------------------------------------------------------|------------------------------------------------------------------------------------------------------------------------------------------|-------------------------------|---------------------------------|---|
| 84    | H                | H                                | H                | H               | C <sub>2</sub> H <sub>5</sub>                                | CH <sub>3</sub>                                                                                                                          | CH <sub>3</sub>               | ClO <sub>4</sub> <sup>⊖</sup>   |   |
| 85    | OCH <sub>3</sub> | OCH <sub>3</sub>                 | H                | CH <sub>3</sub> | (CH <sub>2</sub> ) <sub>3</sub> SO <sub>3</sub> <sup>⊖</sup> | (CH <sub>2</sub> ) <sub>4</sub> SO <sub>3</sub> H.N(C <sub>2</sub> H <sub>5</sub> ) <sub>3</sub>                                         | CH <sub>3</sub>               | —                               |   |
| 86    | H                | COOC <sub>2</sub> H <sub>5</sub> | CF <sub>3</sub>  | H               | C <sub>2</sub> H <sub>5</sub>                                | C <sub>2</sub> H <sub>5</sub>                                                                                                            | C <sub>2</sub> H <sub>5</sub> | I <sup>⊖</sup>                  |   |
| 87    | H                | Cl                               | Cl               | H               | (CH <sub>2</sub> ) <sub>3</sub> SO <sub>3</sub> <sup>⊖</sup> | (CH <sub>2</sub> ) <sub>3</sub> SO <sub>3</sub> H.N(C <sub>2</sub> H <sub>5</sub> ) <sub>3</sub>                                         | C <sub>2</sub> H <sub>5</sub> | —                               |   |
| 88    | H                | Cl                               | Cl               | H               | (CH <sub>2</sub> ) <sub>3</sub> SO <sub>3</sub> <sup>⊖</sup> | C <sub>2</sub> H <sub>5</sub>                                                                                                            | C <sub>2</sub> H <sub>5</sub> | —                               |   |
| 89    | H                | Cl                               | Cl               | H               | (CH <sub>2</sub> ) <sub>4</sub> SO <sub>3</sub> <sup>⊖</sup> | C <sub>2</sub> H <sub>5</sub>                                                                                                            | C <sub>2</sub> H <sub>5</sub> | —                               |   |
| 90    | H                | Cl                               | Cl               | H               | (CH <sub>2</sub> ) <sub>2</sub> COOH                         | (CH <sub>2</sub> ) <sub>3</sub> SO <sub>3</sub> <sup>⊖</sup>                                                                             | C <sub>2</sub> H <sub>5</sub> | —                               |   |
| 91    | H                | OCH <sub>3</sub>                 | H                | H               | (CH <sub>2</sub> ) <sub>4</sub> SO <sub>3</sub> <sup>⊖</sup> | C <sub>2</sub> H <sub>5</sub>                                                                                                            | CH <sub>3</sub>               | —                               |   |
| 92    | H                | OH                               | OH               | H               | (CH <sub>2</sub> ) <sub>3</sub> SO <sub>3</sub> <sup>⊖</sup> | <br>(CH <sub>2</sub> ) <sub>3</sub> SO <sub>3</sub> H.N |                               | C <sub>2</sub> H <sub>5</sub>   |   |
| 93    | H                | CH <sub>3</sub>                  | CH <sub>3</sub>  | H               | (CH <sub>2</sub> ) <sub>3</sub> SO <sub>3</sub> <sup>⊖</sup> | $\begin{array}{c} (\text{CH}_2)_3\text{SO}_3\text{H} \\   \\ (\text{CH}_2)_4\text{SO}_3\text{H.N(C}_2\text{H}_5)_3 \end{array}$          |                               | C <sub>2</sub> H <sub>5</sub>   | — |
| 94    | H                | OCH <sub>3</sub>                 | OCH <sub>3</sub> | H               | (CH <sub>2</sub> ) <sub>4</sub> SO <sub>3</sub> <sup>⊖</sup> | $\begin{array}{c} (\text{CH}_2)_3\text{SO}_3\text{H} \\   \\ (\text{CH}_2)_4\text{SO}_3\text{H.N(C}_2\text{H}_5)_3 \end{array}$          |                               | C <sub>2</sub> H <sub>5</sub>   | — |
| 95    | H                | Cl                               | Cl               | H               | C <sub>2</sub> H <sub>5</sub>                                | $\begin{array}{c} (\text{CH}_2)_2\text{CHSO}_3\text{H} \\   \\ \text{CH}_3 \end{array}$                                                  |                               | C <sub>2</sub> H <sub>5</sub>   | — |

1-96



1-97



I-98



I-99



-continued

I-100



I-101



I-102



I-103



I-104



I-105



-continued

I-106



I-107



I-108



I-109



I-110



I-111



I-112



I-113



I-114



-continued

I-115



I-116



I-117



I-118



I-119



I-120



I-121



I-122



-continued

I-123



I-124



I-125



I-126



I-127



I-128



I-129



I-130



I-131



-continued

I-132



I-133



I-134



I-135



I-136



I-137



I-138



I-139



-continued

I-140

 $I^\ominus$ 

I-141

 $I^\ominus$ 

I-142

 $I^\ominus$ 

I-143

 $I^\ominus$ 

I-144

 $I^\ominus$ 

I-145

 $I^\ominus$ 

I-146

 $I^\ominus$ 

I-147

 $CH_3-C_6H_4-SO_3^\ominus$

-continued

I-148



I-149



I-150



I-151



I-152



I-153



I-154



-continued

I-155



The spectral sensitizers represented by the general formula (I) can be easily synthesized by one skilled in the art if he makes reference to the methods described in various prior art documents including J. Am. Chem. Soc., 67, 1875-1899 (1945), F. M. Hamer, "The Chemistry of Heterocyclic Compounds", Vol. 18, "The Cyanine Dyes and Related Compounds", ed. by A. Weissherger, Interscience, New York, 1964, U.S. Pat. Nos. 3,483,196, 3,541,089, 3,598,595, 3,632,808, 3,757,663, and JP-A-60-78445 (the term "JP-A" as used herein means an "unexamined published Japanese patent application").

Optimal concentrations of the spectral sensitizers represented by the general formula (I) can be determined by any of the methods known to one skilled in the art. According to one method, a given emulsion is divided into two parts, a selected spectral sensitizer is incorporated at different concentrations in the two parts, and the performance of each part of the emulsion is measured to determine an optimum concentration of that emulsion.

The amounts in which the spectral sensitizers of the general formula (I) are to be added are not limited to any particular values but they are preferably used in amounts ranging from  $2 \times 10^{-6}$  to  $1 \times 10^{-2}$  mole per mole of silver halide, with the range of  $5 \times 10^{-6}$  to  $5 \times 10^{-3}$  moles per mole of silver halide being particularly preferred.

The spectral sensitizers of the general formula (I) may be incorporated into emulsions by any of the methods well known in the art. For example, they may be directly incorporated in emulsions. Alternatively, they are first dissolved in water-soluble solvents such as pyridine, methyl alcohol, ethyl alcohol, methyl cellosolve, acetone, fluorinated alcohols, dimethylformamide and mixtures thereof. They may also be diluted with or dissolved in water. The resulting various forms of solution may be added to emulsions. If desired, ultrasonic vibrations may be applied during the preparation of such solutions.

Spectral sensitizers or sensitizing dyes may be incorporated into emulsions by other methods as described in U.S. Pat. No. 3,469,987 (dyes are dissolved in volatile organic solvents, the resulting solution is dispersed in a hydrophilic colloid, and the dispersion thus formed is added to emulsions) and JP-B-46-24185 (the "JP-A" as used herein means an "examined Japanese patent publication") (water-insoluble dyes are dispersed, rather than dissolved in water-soluble solvents, and the resulting dispersion is incorporated in emulsions). Still other methods that can be employed are described in U.S. Pat. Nos. 2,912,345, 3,342,605, 2,996,287, 3,425,835, etc.

The spectral sensitizers of the general formula (I) which are to be used in the present invention may be added to emulsions at any stage of the manufacturing process starting with the formation of silver halide grains and ending just prior to coating on a support. Stated more specifically, the spectral sensitizers may be

15 added at any of the following stages: prior to the formation of silver halide grains; during the formation of silver halide grains; during the period from the end of the formation of silver halide grains to the start of chemical sensitization; at the start of chemical sensitization; during chemical sensitization; at the end of chemical sensitization; and during the period from the end of chemical sensitization to the start of coating operation. If necessary, the sensitizers may be added in divided stages rather than at a time. The order of adding stabilizers and antifoggants is not critical but preferably they are added during the formation of silver halide grains or chemical ripening, namely at a stage prior to the preparation of coating solutions.

20 The spectral sensitizers of the general formula (I) may be combined with either themselves or other spectral sensitizers to achieve supersensitization. In such combinations for supersensitization, the respective spectral sensitizers are dissolved in the same or different solvents and the resulting solutions are added to emulsions either separately or as an admixture. When the solutions are to be added separately, the order of addition and the interval between additions may be determined as appropriate for a specific object.

25 The compounds represented by the general formulas (II) and (III) are described below. Preferred examples of the substituents represented by V<sub>21</sub>, V<sub>22</sub>, V<sub>23</sub> and V<sub>24</sub> include a halogen atom (e.g. Cl), an aryl group (e.g. phenyl), an alkyl group (e.g. preferably C<sub>1-7</sub>, more preferably C<sub>1-4</sub>), an alkoxy group (preferably C<sub>1-6</sub>, more preferably C<sub>1-2</sub>), and an alkoxy carbonyl group (e.g. ethoxycarbonyl). It is also preferred that two adjacent substituents are condensed to form a benzene ring. When Z<sub>3</sub> is



30 a cyano group is also preferably used as V<sub>21</sub>, V<sub>22</sub>, V<sub>23</sub> or V<sub>24</sub>.

35 Preferred examples of the substituents represented by R<sub>21</sub>, R<sub>22</sub>, R<sub>23</sub>, R<sub>24</sub> and R<sub>25</sub> include a halogen atom (e.g. Cl), a hydroxyl group, and an alkyl and an alkoxy group having 1-4 carbon atoms. It is also preferred that two adjacent substituents are condensed to form a ring (e.g. condensed benzene ring or methylenedioxy group).

40 The alkyl group represented by R<sub>26</sub> is preferably an alkyl group having 1-6 carbon atoms such as methyl, ethyl or propyl, and such alkyl groups may have substituents such as an alkoxy group, an alkylthio group, an aryloxy group, an aryl group, a hydroxyl group, a cyano group, a vinyl group, a halogen atom, a carbamoyl group, a sulfamoyl group, a sulfonyl group, an alkoxycarbonyl group, a carboxyl group, etc.

In the general formula (III),  $V_{31}-V_{34}$  have the same meanings as  $V_{21}-V_{24}$ , and  $R_{31}-R_{35}$  also have the same meanings as  $R_{21}-R_{25}$ . Further,  $R_{36}$  has the same meaning as  $R_1$  and  $R_2$ , and  $X_2$  and  $K_2$  have the same meanings as  $X_1$  and  $K_1$ .

The following are specific but non-limiting examples of the compounds that are represented by the general formulas (II) and (III) and which are to be used in the present invention.



| II-No. | V <sub>22</sub>                                                                     | V <sub>23</sub> | R <sub>21</sub> | R <sub>22</sub> | R <sub>23</sub>                                                                     |
|--------|-------------------------------------------------------------------------------------|-----------------|-----------------|-----------------|-------------------------------------------------------------------------------------|
| 1      | H                                                                                   | H               | H               | H               | H                                                                                   |
| 2      | H                                                                                   | H               | H               | H               | Cl                                                                                  |
| 3      | H                                                                                   | H               | H               | H               | OH                                                                                  |
| 4      | H                                                                                   | H               | H               | H               | CH <sub>3</sub>                                                                     |
| 5      | H                                                                                   | H               | H               | H               | OCH <sub>3</sub>                                                                    |
| 6      | H                                                                                   | H               | H               | H               | OC <sub>2</sub> H <sub>5</sub>                                                      |
| 7      | H                                                                                   | H               | H               | H               |    |
| 8      | H                                                                                   | H               | H               | Cl              | H                                                                                   |
| 9      | H                                                                                   | H               | Cl              | H               | H                                                                                   |
| 10     | H                                                                                   | H               | OH              | H               | OH                                                                                  |
| 11     | H                                                                                   | H               | H               | H               | CH <sub>3</sub>                                                                     |
| 12     |  | H               | H               | H               | H                                                                                   |
| 13     |  | H               | Cl              | H               | H                                                                                   |
| 14     | H                                                                                   | H               | H               | H               | Cl                                                                                  |
| 15     | H                                                                                   | H               | H               | H               | OCH <sub>3</sub>                                                                    |
| 16     | H                                                                                   | H               | H               | H               |  |
| 17     | Cl                                                                                  | H               | H               | H               | H                                                                                   |
| 18     | H                                                                                   | H               | H               | H               | Cl                                                                                  |
| 19     | H                                                                                   | H               | H               | H               | CH <sub>3</sub>                                                                     |
| 20     | H                                                                                   | CH <sub>3</sub> | H               | H               | H                                                                                   |



-continued



-continued

II-33



II-34



| II-No. | V <sub>22</sub>  | V <sub>23</sub>  | R <sub>21</sub> | R <sub>22</sub> | R <sub>23</sub>               |
|--------|------------------|------------------|-----------------|-----------------|-------------------------------|
| 35     | H                | H                | H               | H               | H                             |
| 36     | H                | H                | H               | H               | Cl                            |
| 37     | H                | H                | H               | H               | OH                            |
| 38     | H                | H                | H               | H               | OCH <sub>3</sub>              |
| 39     | H                | H                | H               | H               | CH <sub>3</sub>               |
| 40     | Cl               | H                | H               | H               | H                             |
| 41     | Cl               | H                | H               | H               | Cl                            |
| 42     | Cl               | H                | H               | H               | C <sub>2</sub> H <sub>5</sub> |
| 43     | CH <sub>3</sub>  | H                | Cl              | H               | H                             |
| 44     | H                | CH <sub>3</sub>  | OH              | H               | H                             |
| 45     | CH <sub>3</sub>  | CH <sub>3</sub>  | H               | H               | H                             |
| 46     | OCH <sub>3</sub> | H                | H               | H               | H                             |
| 47     | OCH <sub>3</sub> | OCH <sub>3</sub> | H               | H               | H                             |
| 48     |                  |                  |                 |                 |                               |
| 49     | H                | H                | OH              | H               | H                             |
| 50     | H                | H                | H               | OH              | H                             |

II-51



II-52



-continued

II-53



5

II-54



10

II-55



15

II-56



20

II-57



25

II-58



30

II-59



35

II-60



40

II-61



45

II-62



50

-continued

II-63



5

II-64



10

II-65



15

II-66



20

II-67



25

-continued

II-68



II-69



II-70



[III-1]



| III-No. | V <sub>32</sub>                  | V <sub>33</sub> | R <sub>31</sub> | R <sub>32</sub>  | R <sub>33</sub>  | R <sub>36</sub>               | (X <sub>2</sub> )k <sub>2</sub>                              |                |
|---------|----------------------------------|-----------------|-----------------|------------------|------------------|-------------------------------|--------------------------------------------------------------|----------------|
| 1       | H                                |                 | H               | H                | H                | C <sub>2</sub> H <sub>5</sub> | I <sup>⊖</sup>                                               |                |
| 2       | H                                |                 | H               | H                | H                | C <sub>2</sub> H <sub>5</sub> | ClO <sub>4</sub> <sup>⊖</sup>                                |                |
| 3       | H                                |                 | H               | H                | H                | C <sub>2</sub> H <sub>5</sub> | ClO <sub>4</sub> <sup>⊖</sup>                                |                |
| 4       | H                                |                 | H               | H                | H                | OCH <sub>3</sub>              | C <sub>2</sub> H <sub>5</sub>                                | I <sup>⊖</sup> |
| 5       | H                                |                 | H               | H                | H                |                               |                                                              |                |
|         |                                  |                 |                 |                  |                  |                               | BF <sub>4</sub> <sup>⊖</sup>                                 |                |
| 6       | H                                |                 | H               | H                | OCH <sub>3</sub> | H                             |                                                              |                |
| 7       | H                                |                 | H               | OCH <sub>3</sub> | H                | H                             | CH <sub>3</sub>                                              |                |
|         |                                  |                 |                 |                  |                  |                               | CH <sub>3</sub>                                              |                |
| 8       |                                  |                 | H               | H                | H                | H                             | C <sub>2</sub> H <sub>5</sub>                                |                |
|         |                                  |                 |                 |                  |                  |                               | I <sup>⊖</sup>                                               |                |
| 9       | Cl                               |                 | H               | H                | H                | H                             | C <sub>2</sub> H <sub>6</sub>                                |                |
| 10      | COOC <sub>2</sub> H <sub>5</sub> |                 | H               | H                | H                | H                             | C <sub>2</sub> H <sub>6</sub>                                |                |
| 11      |                                  |                 | H               | H                | H                | H                             | —CH <sub>2</sub> —CH=CH—                                     |                |
|         |                                  |                 |                 |                  |                  |                               | I <sup>⊖</sup>                                               |                |
| 12      |                                  |                 | H               | H                | H                | H                             | (CH <sub>2</sub> ) <sub>3</sub> SO <sub>3</sub> <sup>⊖</sup> |                |
|         |                                  |                 |                 |                  |                  |                               | —                                                            |                |

-continued

|    |    |                 |    |   |    |                               |                                                                                    |
|----|----|-----------------|----|---|----|-------------------------------|------------------------------------------------------------------------------------|
| 13 | Cl | CH <sub>3</sub> | H  | H | H  | C <sub>3</sub> H <sub>6</sub> | Br <sup>⊖</sup>                                                                    |
| 14 | H  | H               | Cl | H | Cl | CH <sub>3</sub>               |  |

15      CH<sub>3</sub>      H      H      Cl      CH<sub>3</sub>      I<sup>⊖</sup>  
 III-16      



III-17



III-18



III-19



III-2

| III-No. | V <sub>32</sub>  | V <sub>33</sub> | R <sub>31</sub>  | R <sub>32</sub> | R <sub>33</sub>                | R <sub>36</sub>                                              | (X <sub>2</sub> )k <sub>2</sub> |
|---------|------------------|-----------------|------------------|-----------------|--------------------------------|--------------------------------------------------------------|---------------------------------|
| 20      | H                | H               | H                | H               | H                              | C <sub>2</sub> H <sub>5</sub>                                | I <sup>Θ</sup>                  |
| 21      | H                | H               | H                | H               | Cl                             | C <sub>2</sub> H <sub>5</sub>                                | I <sup>Θ</sup>                  |
| 22      | H                | H               | H                | H               | OH                             | C <sub>2</sub> H <sub>5</sub>                                | I <sup>Θ</sup>                  |
| 23      | H                | H               | H                | H               | CH <sub>3</sub>                | C <sub>2</sub> H <sub>5</sub>                                | I <sup>Θ</sup>                  |
| 24      | H                | H               | H                | H               | C <sub>2</sub> H <sub>5</sub>  | C <sub>2</sub> H <sub>5</sub>                                | I <sup>Θ</sup>                  |
| 25      | H                | H               | OCH <sub>3</sub> | H               | OCH <sub>3</sub>               | C <sub>2</sub> H <sub>5</sub>                                | I <sup>Θ</sup>                  |
| 26      | CH <sub>3</sub>  | H               | H                | H               | H                              | CH <sub>3</sub>                                              | ClO <sub>4</sub> <sup>Θ</sup>   |
| 27      | H                | CH <sub>3</sub> | H                | H               | H                              | CH <sub>3</sub>                                              | ClO <sub>4</sub> <sup>Θ</sup>   |
| 28      | CH <sub>3</sub>  | CH <sub>3</sub> | H                | H               | H                              | CH <sub>3</sub>                                              | ClO <sub>4</sub> <sup>Θ</sup>   |
| 29      | OCH <sub>3</sub> | H               | H                | H               | H                              | CH <sub>3</sub>                                              | ClO <sub>4</sub> <sup>Θ</sup>   |
| 30      | Cl               | H               | H                | H               | H                              | C <sub>2</sub> H <sub>5</sub>                                | ClO <sub>4</sub> <sup>Θ</sup>   |
| 31      | Cl               | H               | H                | H               | Cl                             | C <sub>2</sub> H <sub>5</sub>                                | ClO <sub>4</sub> <sup>Θ</sup>   |
| 32      | Cl               | H               | H                | Cl              | H                              | C <sub>2</sub> H <sub>5</sub>                                | ClO <sub>4</sub> <sup>Θ</sup>   |
| 33      | Cl               | H               | H                | H               | H                              | (CH <sub>2</sub> ) <sub>4</sub> SO <sub>4</sub> <sup>Θ</sup> | —                               |
| 34      | Cl               | H               | H                | H               | OC <sub>2</sub> H <sub>5</sub> | CH <sub>3</sub>                                              | I <sup>Θ</sup>                  |

-continued

III-35

 $\text{I}^\ominus$ 

III-36

 $\text{ClO}_4^\ominus$ 

III-37

 $\text{I}^\ominus$ 

III-38

 $\text{I}^\ominus$ 

III-39

 $(\text{CH}_2)_3\text{SO}_4^\ominus$ 

III-40

 $\text{Br}^\ominus$ 

III-41

 $\text{CH}_3\text{---C}_6\text{H}_4\text{---SO}_3^\ominus$ 

III-42

 $\text{CH}_3\text{---C}_6\text{H}_4\text{---SO}_3^\ominus$

-continued

III-43



III-44



III-45



The compounds represented by the general formula (II) or (III) are preferably used in sufficient amounts to achieve supersensitization. It is particularly preferred to use them in amounts ranging from  $1 \times 10^{-8}$  to  $1 \times 10^{-2}$  mole per mole of silver halide in an emulsion.

The molar ratio of the spectral sensitizer of the general formula (I) to the compound of the general formula (II) or (III) is preferably within the range of 10:1 to 1:100, with the range of 2:1 to 1:10 being particularly preferred.

The compounds of the general formula (II) or (III) may be dispersed directly in an emulsion. Alternatively, they may be added to the emulsion after being dissolved in a suitable solvent (e.g. methyl alcohol, ethyl alcohol, methyl cellosolve or water) or a mixed solvent system consisting two or more of those solvents.

It is also possible to add the compounds of (II) or (III) in the form of either a solution or a dispersion in colloid in accordance with customary methods of addition of spectral sensitizers.

The compounds represented by the general formula (II) or (III) may be added simultaneously with or separately from the spectral sensitizers represented by the general formula (I). Preferably, those compounds are added simultaneously with the spectral sensitizers of the general formula (I).

The silver halide grains incorporated in the silver halide photographic material of the present invention may have any halide composition such as silver bromide, silver chloride, silver chlorobromide, silver iodobromide or silver chloroiodobromide. Silver iodobromide is particularly preferred since it provides high sensitivity. In the case of silver iodobromide, the average content of silver iodide in the grains is preferably in the range of 0.5-10 mol %, with the range of 1-8 mol % being more preferred.

The objects of the present invention can be attained more effectively if the silver halide grains incorporated in at least one silver halide emulsion layer which are spectrally sensitized with the dyes of the general formula (I) are adapted to have a core/shell structure. Grains having a core/shell structure are such that the core of a grain is surrounded with a shell having a different composition. In grains having a core/shell structure, the shell may be homogeneous but preferably, a

25 shell on the core is coated with another shell having a different silver halide composition to produce a multi-layered shell structure.

If silver halide crystals having a silver iodobromide (or silver chloroiodobromide) core/shell structure are 30 to be used in the present invention, the silver iodide content of the shell preferably ranges from 2 to 40 mol %, with the range of 10-40 mol % being more preferred. The most preferred range is from 15 to 40 mol %.

35 In preparing silver halide crystals composed of silver iodobromide (or silver chloroiodobromide), iodide ions may be added either as an ionic solution such as a potassium iodide solution or as grains having a smaller solubility product than growing silver halide grains. Preferably, iodide ions are added as silver halide grains having a smaller solubility product than growing silver halide grains.

40 The silver halide grains to be used in the present invention may be "normal crystals" having a cubic, octahedral, tetrahedral or spherical shape; alternatively, they may be crystals containing twins. The processes for preparing silver halide grains in the form of normal crystal are known and are described in references such as J. Phot. Sci., 5, 332 (1961), Ber. Bunsenges. Phys. Chem., 67, 949 (1963) and Intern. Congress of Phot. Sci., Tokyo (1967).

45 Tabular grains having aspect ratios of 5 or more may also be used in the present invention. Tabular grains can be easily prepared by the methods described in U. S. Pat. Nos. 4,434,226, 4,414,310, 4,433,048, 4,439,520, U.K. Pat. No. 2,112,157, etc. Tabular grains for use in the present invention preferably have aspect ratios of 5-100, more preferably 5-20. Such tabular grains preferably have a size of 0.2-30  $\mu\text{m}$ , more preferably 0.4-10  $\mu\text{m}$ , in terms of the diameter of an equivalent circle. Their thickness is preferably 0.5  $\mu\text{m}$  or below, more preferably 0.3  $\mu\text{m}$  or below.

50 The silver halide emulsions to be used in the present invention may be polydispersed but, more preferably, monodispersed emulsions are used. The term "monodispersed emulsions" as used herein means such silver halide emulsions that at least 95% of the grains are within  $\pm 40\%$ , preferably  $\pm 30\%$ , of the average grain

size in terms of either number or weight when the average grain diameter is measured by the method reported by A. P. H. Trivelli and W. F. Smith in *The Photographic Journal*, 79, 330-338 (1939).

The above-described silver halide grains to be used in the silver halide photographic material of the present invention can be prepared by the various methods described in T. H. James, "The Theory of the Photographic Process", Fourth Edition, pp. 38-104, Macmillan Publishing Co., New York (1977), including the neutral method, the acid method, the ammoniacal method normal precipitation, reverse precipitation, the double-jet method, the controlled double-jet method, the conversion method, and the core/shell method.

Known photographic additives can be added to the silver halide photographic emulsions for in the present invention. Exemplary photographic additives are the following compounds described in Research Disclosure (RD) Item 17643 and Item 18716.

| Additive                | RD-17643         | RD-18716                                        |
|-------------------------|------------------|-------------------------------------------------|
| Chemical sensitizer     | page 23, III     | page 648, upper right column                    |
| Development accelerator | page 29, XXI     | page 648, upper right column                    |
| Antifoggent             | page 24, VI      | page 649, lower right column                    |
| Stabilizer              | page 24, VI      | page 649, lower right column                    |
| Anti-color stain agent  | page 25, VII     | page 650, left and right columns                |
| Image stabilizer        | page 25, VII     | page 649, right column to page 650, left column |
| UV Absorber             | pages 25-26, VII | page 649, right column to page 650, left column |
| Filter dye              | pages 25-26, VII | page 649, right column to page 650, left column |
| Brightening agent       | page 24, V       | page 651, right column                          |
| Hardener                | page 26, X       | page 651, right column                          |
| Coating aid             | pages 26-27, XI  | page 650, right column                          |
| Surfactant              | pages 26-27, XI  | page 650, right column                          |
| Plasticizer             | page 27, XII     | page 650, right column                          |
| Slip agent              | page 27, XII     | page 650, right column                          |
| Antistatic agent        | page 27, XII     | page 650, right column                          |
| Matting agent           | page 28, XVI     | page 650, right column                          |
| Binder                  | page 26, IX      | page 651, right column                          |

The photographic material of the present invention can be processed using dye forming couplers that are capable of forming dyes upon coupling with the oxidation products of aromatic primary amino developing agents such as p-phenylenediamine derivatives and aminophenol derivatives. The dye forming couplers are usually selected in such a way as to form dyes that absorb spectral light to which the emulsion layers containing those couplers have sensitivity. Stated more specifically, yellow dye forming couplers are used in a blue-sensitive emulsion layer, magenta dye forming couplers in a green-sensitive emulsion layer, and cyan dye forming couplers in a red-sensitive emulsion layer. However, the silver halide color photographic material of the present invention may adopt other combinations of dye forming couplers and emulsion layers depending on a specific abject.

The dye forming couplers to be used in the present invention desirably have "ballast" groups in their molecules, which "ballast groups" are groups with 8 or more carbon atoms that render the couplers non-diffusible.

- 5 The dye forming couplers may be of a four-equivalent type which requires four molecules of silver ion to be reduced in order to form a molecule of dye, or they may be of a two-equivalent type which requires only two molecules of silver ion to be reduced in order to form a

10 molecule of dye. Included within the category of dye forming couplers are colored couplers which are capable of color correction, as well as compounds that, upon coupling with the oxidation products of developing agents, release photographically useful fragments such

15 as a development restrainer, a development accelerator, a bleach accelerator, a developing agent, a silver halide solvent, a toning agent, a hardener, a foggant, an anti-foggant, a chemical sensitizer, a spectral sensitizer and a desensitizer. Among these couplers and compounds,

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455 10460 10465 10470 10475 10480 10485 10490 10495 10500 10505 10510 10515 10520 10525 10530 10535 10540 10545 10550 10555 10560 10565 10570 10575 10580 10585 10590 10595 10600 10605 10610 10615 10620 10625 10630 10635 10640 10645 10650 10655 10660 10665 10670 10675 10680 10685 10690 10695 10700 10705 10710 10715 10720 10725 10730 10735 10740 10745 10750 10755 10760 10765 10770 10775 10780 10785 10790 10795 10800 10805 10810 10815 10820 10825 10830 10835 10840 10845 10850 10855 10860 10865 10870 10875 10880 10885 10890 10895 10900 10905 10910 10915 10920 10925 10930 10935 10940 10945 10950 10955 10960 10965 10970 10975 10980 10985 10990 10995 11000 11005 11010 11015 11020 11025 11030 11035 11040 11045 11050 11055 11060 11065 11070 11075 11080 11085 11090 11095 11100 11105 11110 11115 11120 11125 11130 11135 11140 11145 11150 11155 11160 11165 11170 11175 11180 11185 11190 11195 11200 11205 11210 11215 11220 11225 11230 11235 11240 11245 11250 11255 11260 11265 11270 11275 11280 11285 11290 11295 11300 11305 11310 11315 11320 11325 11330 11335 11340 11345 11350 11355 11360 11365 11370 11375 11380 11385 11390 11395 11400 11405 11410 11415 11420 11425 11430 11435 11440 11445 11450 11455 11460 11465 11470 11475 11480 11485 11490 11495 11500 11505 11510 11515 11520 11525 11530 11535 11540 11545 11550 11555 11560 11565 11570 11575 11580 11585 11590 11595 11600 11605 11610 11615 11620 11625 11630 11635 11640 11645 11650 11655 11660 11665 11670 11675 11680 11685 11690 11695 11700 11705 11710 11715 11720 11725 11730 11735 11740 11745 11750 11755 11760 11765 11770 11775 11780 11785 11790 11795 11800 11805 11810 11815 11820 11825 11830 11835 11840 11845 11850 11855 11860 11865 11870 11875 11880 11885 11890 11895 11900 11905 11910 11915 11920 11925 11930 11935 11940 11945 11950 11955 11960 11965 11970 11975 11980 11985 1199

Known acylacetanilide containing couplers can preferably be used as yellow-dye forming couplers. Among them, benzoylacetanilide and pivaloylacetanilide containing compounds are advantageous.

- 50 Specific examples of the yellow color forming couplers that can be used are described U.S. Pat. Nos. 2,875,057, 3,265,506, 3,408,194, 3,551,155 3,582,322, 3,725,072, 3,891,445, German Patent No. 1,547,868, German Patent Application (OLS) Nos. 2,219,917,  
55 2,261,361, 2,414,006, U.K. Patent No. 1,425,020, JP-B-51-10783, JP-A-47-26133, JP-A-48-73147, JP-A-50-6341, JP-A-50-87650, JP-A-50-123342, JP-A-50-130442, JP-A-51-21827, JP-A-51-102636, JP-A-52-82424, JP-A-52-115219, JP-A-58-95346, etc.

60 Pyrazolone-, indazolone- and cyanoacetyl-containing compounds can be used as magenta color forming couplers, with pyrazolone-containing compounds being particularly advantageous.

- Specific examples of the magenta color forming couplers that can be used are described in U.S. Pat. Nos. 2,600,788, 2,983,608, 3,062,653, 3,127,269, 3,311,476, 3,419,391, 3,519,429, 3,558,319, 3,582,322, 3,615,506, 3,834,908, 3,891,445, German Patent No. 1,810,464.

German Patent Application (OLS) Nos. 2,408,665, 2,417,945, 2,418,959, 2,424,467, JP-B-40-6031, JP-A-51-20826, JP-A-52-58922, JP-A-49-129538, JP-A-49-74027, JP-A-50-159336, JP-A-52-42121, JP-A-49-74028, JP-A-50-60233, JP-A-51-26541, JP-A-53-55122, JP-A-59-171956, JP-A-60-35552, JP-A-60-43659, JP-A-60-172982, JP-A-60-190779, etc.

Phenolic and naphtholic compounds can be used as cyan color forming couplers. Specific examples of the cyan color forming couplers that can be used are described in U.S. Pat. Nos. 2,369,929, 2,434,272, 2,474,293, 2,521,908, 2,895,826, 3,034,892, 3,311,476, 3,458,315, 3,476,563, 3,583,971, 3,591,383, 3,767,411, 4,004,929, German Patent Application (OLS) Nos. 2,414,830, 2,454,329, JP-A-48-59838, JP-A-51-26034, JP-A-48-5055, JP-A-51-146828, JP-A-52-69624, etc.

The silver halide photographic material of the present invention can be produced by coating emulsion layers and other necessary photographic layers on supports that have a high degree of flatness and that are dimensionally stable during both production and subsequent photographic processing. Suitable supports include, for example, a nitryl cellulose film, a cellulose ester film, a polyvinyl acetal film, a polystyrene film, a polyethylene terephthalate film, a polycarbonate film, glass, paper, metals, as well as paper coated with polyolefins such as polyethylene and polypropylene. These supports may be subjected to various surface treatments such as one for rendering their surface hydrophilic in order to improve the adhesion to photographic layers such as emulsion layers. Examples of such surface treatments are halogenation, corona discharge treatment, subbing treatment and setting treatment.

The silver halide color photographic material of the present can be processed using known processing solutions by known photographic processing methods as described in Research Disclosure No. 176 (RD-17643), pp. 20-30. The temperature to be used in the photographic processing is usually in the range of 18°-50° C. It should, however, be noted that the photographic material of the present invention can be processed at temperatures either lower than 18° C. or higher than 50° C.

The silver halide color photographic material of the present invention can be applied to various light-sensitive materials including color negative films for picture taking, color reversal films, color papers, color positive films, color reversal papers, direct positive camera materials, heat-processable light-sensitive materials, and silver dye bleachable light-sensitive materials.

The following examples are provided for the purpose of further illustrating the present invention but are in no way to be taken as limiting. In the examples that follow, the amounts of components or additives in silver halide photographic materials are based on one square meter unless otherwise noted. The amounts of silver halides and colloidal silver are calculated for silver. The amounts of spectral sensitizers are expressed in moles per mole of silver. The structures of the compounds used in the examples are collectively shown at the end of Example 4.

#### EXAMPLE 1

##### Preparation of sample No. 101

A silver iodobromide emulsion having an average grain size of 0.4  $\mu$ m and a core with a AgI content of 15 mol % (average AgI content, 8 mol %) was subjected to optimal gold-plus-sulfur sensitization. Thereafter, the

emulsion was spectrally sensitized to green by adding illustrative sensitizing dyes I-35 and I-50 in respective amounts of  $4.5 \times 10^{-4}$  and  $3 \times 10^{-4}$  moles per mole of silver. Then, the emulsion was stabilized by addition of 4-hydroxy-6-methyl-1,3,3a,7-tetraazaindene and 1-phenyl-5-mercaptotetrazole.

Subsequently, a magenta coupler (M-1) was dissolved in ethyl acetate and dinonyl phthalate (DNP) and the solution was dispersed in an aqueous solution containing gelatin. Then, customary photographic additives including a spreading agent and a hardener were added to the dispersion, thereby preparing an emulsion coating solution. This coating solution was applied onto a subbed triacetyl cellulose base in the usual manner and dried to prepare a light-sensitive material sample No. 101.

##### Preparation of sample Nos. 102-115

Sample Nos. 102-115 were prepared by repeating the procedure of preparing sample No. 101 except that the compounds listed in Table 1 were added to the spectral sensitizer used in sample No. 101.

Sample Nos. 101-115 were subjected to wedge exposure in the usual manner and subsequently processed by the following scheme.

| Steps (at 38° C.)  | Time             |
|--------------------|------------------|
| Color development  | 3 min and 15 sec |
| Bleaching          | 6 min and 30 sec |
| Washing with water | 3 min and 15 sec |
| Fixing             | 6 min and 30 sec |
| Washing with water | 3 min and 15 sec |
| Stabilizing        | 1 min and 30 sec |

The processing solutions used in the color developing, bleaching, fixing and stabilizing steps had the following compositions.

| Color developing solution                                          |                  |
|--------------------------------------------------------------------|------------------|
| 4-Amino-3-methyl-N-ethyl-N-( $\beta$ -hydroxyethyl)aniline sulfate | 4.75 g           |
| Anhydrous sodium sulfite                                           | 4.25 g           |
| Hydroxylamine sulfate                                              | 2.0 g            |
| Anhydrous potassium carbonate                                      | 37.5 g           |
| Potassium bromide                                                  | 1.3 g            |
| Nitrotriacetic acid trisodium salt (monohydrate)                   | 2.5 g            |
| Potassium hydroxide                                                | 1.0 g            |
| Water                                                              | to make 1,000 ml |
| Bleaching solution                                                 |                  |
| Ethylenediaminetetraacetic acid                                    | 100.0 g          |
| iron ammonium salt                                                 |                  |
| Ethylenediaminetetraacetic acid                                    | 10.0 g           |
| diammonium salt                                                    |                  |
| Ammonium bromide                                                   | 150.0 g          |
| Glacial acetic acid                                                | 10.0 ml          |
| Water                                                              | to make 1,000 ml |
| pH                                                                 | adjusted to 6.0  |
|                                                                    | with             |
|                                                                    | aqueous ammonia  |
| Fixing solution                                                    |                  |
| Ammonium thiosulfate                                               | 175.0 g          |
| Anhydrous sodium sulfite                                           | 8.6 g            |
| Sodium metasulfite                                                 | 2.3 g            |
| Water                                                              | to make 1,000 ml |
| pH                                                                 | adjusted to 6.0  |
|                                                                    | with             |
|                                                                    | acetic acid      |
| Stabilizing solution                                               |                  |
| Formaldehyde (37% aq. sol.)                                        | 1.5 ml           |
| Konidax (product of Konica Corp.)                                  | 7.5 ml           |
| Water                                                              | to make 1,000 ml |

The fog, sensitivity and raw stock stability of sample Nos. 101-115 were evaluated by the following procedures and the results are shown in Table 1.

Sensitivity: Expressed as the reciprocal of the amount of exposure necessary to impart fog (min. density +0.1. The results are indicated in relative values, with the value for sample No. 101 being taken as 100.

Raw stock stability: Samples as prepared by coating emulsion layers were left to stand for 3 days either under natural conditions (run C) or at a temperature of 50° C. and 80% r.h. (run D under accelerated aging conditions). The sensitivity of run D to green light as compared to the sensitivity of run C was expressed in relative values, with the value for run C being taken as 100. The higher the value of D/C, the better the raw stock stability of samples.

TABLE 1

| Sample No. | Compound | Amount (mol/mol AgX) | Fog                  | Sensitivity | Raw stock stability |
|------------|----------|----------------------|----------------------|-------------|---------------------|
| Comparison | 101      | —                    | —                    | 0.16        | 100                 |
|            | 102      | CR-1                 | $7.5 \times 10^{-5}$ | 0.25        | 84                  |
|            | 103      | CR-3                 | $7.5 \times 10^{-5}$ | 0.22        | 89                  |
|            | 104      | CR-4                 | $7.5 \times 10^{-5}$ | 0.35        | 41                  |
| Invention  | 105      | II-1                 | $7.5 \times 10^{-5}$ | 0.12        | 153                 |
|            | 106      | II-2                 | $7.5 \times 10^{-5}$ | 0.12        | 159                 |
|            | 107      | II-5                 | $7.5 \times 10^{-5}$ | 0.13        | 149                 |
|            | 108      | II-36                | $7.5 \times 10^{-5}$ | 0.12        | 142                 |
|            | 109      | II-37                | $7.5 \times 10^{-5}$ | 0.13        | 135                 |
|            | 110      | II-38                | $7.5 \times 10^{-5}$ | 0.14        | 139                 |
|            | 111      | II-39                | $7.5 \times 10^{-5}$ | 0.13        | 138                 |
|            | 112      | II-40                | $7.5 \times 10^{-5}$ | 0.13        | 134                 |
|            | 113      | II-65                | $7.5 \times 10^{-5}$ | 0.14        | 134                 |
|            | 114      | III-1                | $7.5 \times 10^{-5}$ | 0.15        | 138                 |
|            | 115      | III-44               | $7.5 \times 10^{-5}$ | 0.15        | 131                 |

As is clear from Table 1, the samples of the present invention had low fog and were improved in terms of sensitivity and the storage stability of raw stock (i.e. samples just after preparation).

## EXAMPLE 2

## Preparation of Sample No. 201

A silver iodobromide emulsion having an average grain size of 0.4  $\mu\text{m}$  and an average AgI content of 2 mol % was subjected to optimal gold-plus-sulfur sensitization. Thereafter, the emulsion was spectrally sensitized by addition of a sensitizing dye I-10 in an amount of  $5.8 \times 10^{-4}$  moles per mole of silver. Then, the emul-

tives including a spreading agent and a hardener were added to the dispersion, thereby preparing an emulsion coating solution. This coating solution was applied onto a subbed triacetyl cellulose base in the usual manner and dried to prepare a light-sensitive material sample No. 201.

## Preparation of Sample Nos. 202-208

Sample Nos. 202-208 were prepared by repeating the procedure of preparing sample No. 201 except that the compounds listed in Table 2 were added to the spectral sensitizer I-10 used in sample No. 201.

## Preparation of Sample Nos. 209-212

Sample Nos. 209-212 were prepared by repeating the procedure of preparing sample Nos. 205-208 except

that the emulsion used was replaced by a silver iodobromide emulsion having an average grain size of 0.4  $\mu\text{m}$  and a core with 15 mol % AgI (average AgI content, 8 mol %).

Sample Nos. 201-212 were subjected to wedge exposure in the usual manner and subsequently processed as in Example 1.

The fog, sensitivity, and raw stock stability of sample Nos. 201-212 were evaluated as in Example 1. The results are shown in Table 2, in which the sensitivity is expressed in relative values, with the value for sample No. 201 being taken as 100, and both sensitivity and raw stock stability are related to blue light.

TABLE 2

| Sample No. | Compound | Amount (mol/mol AgX) | Fog                  | Sensitivity | Raw stock stability |
|------------|----------|----------------------|----------------------|-------------|---------------------|
| Comparison | 201      | —                    | —                    | 0.15        | 100                 |
|            | 202      | CR-2                 | $5.8 \times 10^{-5}$ | 0.18        | 109                 |
|            | 203      | CR-5                 | $5.8 \times 10^{-5}$ | 0.42        | 28                  |
| Invention  | 204      | II-3                 | $5.8 \times 10^{-5}$ | 0.14        | 131                 |
|            | 205      | II-35                | $5.8 \times 10^{-5}$ | 0.13        | 140                 |
|            | 206      | II-36                | $5.8 \times 10^{-5}$ | 0.13        | 145                 |
|            | 207      | II-51                | $5.8 \times 10^{-5}$ | 0.12        | 138                 |
|            | 208      | III-20               | $5.8 \times 10^{-5}$ | 0.15        | 137                 |
|            | 209      | II-35                | $5.8 \times 10^{-5}$ | 0.14        | 181                 |
|            | 210      | II-36                | $5.8 \times 10^{-5}$ | 0.13        | 187                 |
|            | 211      | II-51                | $5.8 \times 10^{-5}$ | 0.13        | 180                 |
|            | 212      | III-20               | $5.8 \times 10^{-5}$ | 0.14        | 176                 |

sion was stabilized by addition of 4-hydroxy-6-methyl-1,3,3a,7-tetraazaindene and 1-phenyl-5-mercaptopetrazole.

Subsequently, a yellow coupler (Y-1) was dissolved in ethyl acetate and tricresyl phosphate (TCP) and the resulting solution was dispersed in an aqueous solution containing gelatin. Then, customary photographic addi-

As is clear from Table 2, the samples of the present invention had low fog and were improved in terms of sensitivity and raw stock stability. Further, comparing sample Nos. 205-208 with sample Nos. 209-212, one can see that further improvements in sensitivity and raw

stock stability could be attained in the present invention by using a core/shell type emulsion.

### EXAMPLE 3

#### Preparation of sample No. 301

A silver iodobromide emulsion having an average grain size of  $0.4 \mu\text{m}$  and a core with a  $\text{AgI}$  content of 15 mol % (average  $\text{AgI}$  content, 8 mol %) was subjected to optimal gold-plus-sulfur sensitization. Thereafter, the emulsion was spectrally sensitized to red by adding illustrative sensitizing dyes I-87, I-107 and I-98 in respective amounts of  $3.2 \times 10^{-4}$ ,  $3.2 \times 10^{-4}$  and  $0.4 \times 10^{-4}$  moles per mole of silver. Then, the emulsion was stabilized by addition of 4-hydroxy-6-methyl-1,3,3a,7-tetrazaindene and 1-phenyl-5-mercaptopotetrazole.

Subsequently, a cyan coupler (C-1) was dissolved in

dried to prepare a light-sensitive material sample No. 301.

#### Preparation of sample Nos. 302-310

5 Sample Nos. 302-310 were prepared by repeating the procedure of preparing sample No. 301 except that the compounds listed in Table 3 were added to the spectral sensitizer used in sample No. 301.

10 Sample Nos. 301-310 were subjected to wedge exposure in the usual manner and subsequently processed as in Example 1.

15 The fog, sensitivity and raw stock stability of sample Nos. 301-310 were evaluated as in Example 1. The results are shown in Table 3, in which the sensitivity is expressed in relative values, with the value for sample No. 301 being taken as 100, and both sensitivity and raw stock stability are related to red light.

TABLE 3

| Sample No.      | Compound | Amount (mol/mol AgX)  | Fog  | Sensitivity | Raw stock stability |
|-----------------|----------|-----------------------|------|-------------|---------------------|
| Compar-<br>ison | 301      | —                     | —    | 100         | 70                  |
|                 | 302      | $6.8 \times 10^{-5}$  | 0.19 | 104         | 64                  |
|                 | 303      | $6.8 \times 10^{-5}$  | 0.21 | 103         | 61                  |
|                 | 304      | $13.6 \times 10^{-5}$ | 0.35 | 84          | 59                  |
|                 | 305      | $6.8 \times 10^{-5}$  | 0.25 | 85          | 59                  |
| Inven-<br>tion  | 306      | $6.8 \times 10^{-5}$  | 0.12 | 138         | 84                  |
|                 | 307      | $13.6 \times 10^{-5}$ | 0.13 | 139         | 82                  |
|                 | 308      | $6.8 \times 10^{-5}$  | 0.14 | 136         | 80                  |
|                 | 309      | $6.8 \times 10^{-5}$  | 0.14 | 134         | 79                  |
|                 | 310      | $6.8 \times 10^{-5}$  | 0.15 | 135         | 76                  |

ethyl acetate and dinonyl phthalate (DNP) and the solution was dispersed in an aqueous solution containing gelatin. Then, customary photographic additives including a spreading agent and a hardener were added to the dispersion, thereby preparing an emulsion coating solution. This coating solution was applied onto a subbed triacetyl cellulose base in the usual manner and

As is clear from Table 3, the samples of the present invention had low fog and were improved in terms of sensitivity and raw stock stability.

### EXAMPLE 4

#### Preparation of Sample No. 401

35 Multi-layered color photographic element sample No. 401 was prepared by forming the following layers in the order written on a triacetyl cellulose film base.

|                                                                |                                   |
|----------------------------------------------------------------|-----------------------------------|
| <u>First layer: Anti-halo layer (HC)</u>                       |                                   |
| Black colloidal silver                                         | 0.15                              |
| UV Absorber (UV-1)                                             | 0.20                              |
| Colored cyan coupler (CC-1)                                    | 0.02                              |
| High-boiling Point solvent (Oil-1)                             | 0.20                              |
| High-boiling point solvent (Oil-2)                             | 0.20                              |
| Gelatin                                                        | 1.6                               |
| <u>Second layer: Intermediate layer (IL-1)</u>                 |                                   |
| Gelatin                                                        | 1.3                               |
| <u>Third layer: Less red-sensitive emulsion layer (R-L)</u>    |                                   |
| Silver iodobromide emulsion (Em-1)                             | 0.4                               |
| Silver iodobromide emulsion (Em-2)                             | 0.3                               |
| Sensitizing dye (I-87)                                         | $3.2 \times 10^{-4}$ (mol/mol Ag) |
| Sensitizing dye (I-107)                                        | $3.2 \times 10^{-4}$ (mol/mol Ag) |
| Sensitizing dye (I-98)                                         | $0.2 \times 10^{-4}$ (mol/mol Ag) |
| Cyan coupler (C-1)                                             | 0.50                              |
| Cyan coupler (C-2)                                             | 0.13                              |
| Colored cyan coupler (CC-1)                                    | 0.07                              |
| DIR compound (D-1)                                             | 0.006                             |
| DIR compound (D-2)                                             | 0.01                              |
| High-boiling point solvent (Oil-1)                             | 0.55                              |
| Gelatin                                                        | 1.0                               |
| <u>Fourth layer: Highly red-sensitive emulsion layer (R-H)</u> |                                   |
| Silver iodobromide emulsion (Em-3)                             | 0.9                               |
| Sensitizing dye (I-87)                                         | $1.7 \times 10^{-4}$ (mol/mol Ag) |
| Sensitizing dye (I-107)                                        | $1.6 \times 10^{-4}$ (mol/mol Ag) |
| Sensitizing dye (I-98)                                         | $0.1 \times 10^{-4}$ (mol/mol Ag) |
| Cyan coupler (C-2)                                             | 0.23                              |
| Colored cyan coupler (CC-1)                                    | 0.03                              |
| DIR compound (D-2)                                             | 0.02                              |
| High-boiling point solvent Oil-1                               | 0.25                              |
| Gelatin                                                        | 1.0                               |

-continued

|                                                                    |                                   |
|--------------------------------------------------------------------|-----------------------------------|
| <u>Fifth layer: Intermediate layer (IL-2)</u>                      |                                   |
| Gelatin                                                            | 0.8                               |
| <u>Sixth layer: Less green-sensitive emulsion layer (G-L)</u>      |                                   |
| Silver iodobromide emulsion (Em-1)                                 | 0.6                               |
| Silver iodobromide emulsion (Em-2)                                 | 0.2                               |
| Sensitizing dye (I-39)                                             | $0.7 \times 10^{-4}$ (mol/mol Ag) |
| Sensitizing dye (I-60)                                             | $0.8 \times 10^{-4}$ (mol/mol Ag) |
| Magenta coupler (M-1)                                              | 0.17                              |
| Magenta coupler (M-2)                                              | 0.43                              |
| Colored Magenta coupler (CM-1)                                     | 0.10                              |
| DIR compound (D-3)                                                 | 0.02                              |
| High-boiling point solvent (Oil-2)                                 | 0.7                               |
| Gelatin                                                            | 1.0                               |
| <u>Seventh layer: Highly green-sensitive emulsion layer (G-H)</u>  |                                   |
| Silver iodobromide emulsion (Em-3)                                 | 0.9                               |
| Sensitizing dye (I-50)                                             | $1.1 \times 10^{-4}$ (mol/mol Ag) |
| Sensitizing dye (I-35)                                             | $2.0 \times 10^{-4}$ (mol/mol Ag) |
| Sensitizing dye (I-40)                                             | $0.3 \times 10^{-4}$ (mol/mol Ag) |
| Magenta coupler (M-1)                                              | 0.03                              |
| Magenta coupler (M-2)                                              | 0.13                              |
| Colored magenta coupler (CM-1)                                     | 0.04                              |
| DIR compound (D-3)                                                 | 0.004                             |
| High-boiling point solvent (Oil-2)                                 | 0.35                              |
| Gelatin                                                            | 1.0                               |
| <u>Eighth layer: Yellow filter layer (YC)</u>                      |                                   |
| Yellow colloidal silver                                            | 0.1                               |
| Additive (SC-1)                                                    | 0.12                              |
| Additive (HS-1)                                                    | 0.07                              |
| Additive (HS-2)                                                    | 0.07                              |
| High-boiling point solvent (Oil-2)                                 | 0.15                              |
| Gelatin                                                            | 1.0                               |
| <u>Ninth layer: Less blue-sensitive emulsion layer (B-L)</u>       |                                   |
| Silver iodobromide emulsion (Em-1)                                 | 0.25                              |
| Silver iodobromide emulsion (Em-2)                                 | 0.25                              |
| Sensitizing dye (I-10)                                             | $5.8 \times 10^{-4}$ (mol/mol Ag) |
| Yellow coupler (Y-1)                                               | 0.60                              |
| Yellow coupler (Y-2)                                               | 0.32                              |
| DIR compound (D-1)                                                 | 0.003                             |
| DIR compound (D-2)                                                 | 0.006                             |
| High-boiling point solvent (Oil-2)                                 | 0.18                              |
| Gelatin                                                            | 1.3                               |
| <u>Tenth layer: Highly blue-sensitive emulsion layer (B-H)</u>     |                                   |
| Silver iodobromide emulsion (Em-4)                                 | 0.5                               |
| Sensitizing dye (I-3)                                              | $3.0 \times 10^{-4}$ (mol/mol Ag) |
| Sensitizing dye (I-17)                                             | $1.2 \times 10^{-4}$ (mol/mol Ag) |
| Yellow coupler (Y-1)                                               | 0.18                              |
| Yellow coupler (Y-2)                                               | 0.10                              |
| High-boiling point solvent (Oil-2)                                 | 0.05                              |
| Gelatin                                                            | 1.0                               |
| <u>Eleventh layer: First protective layer (PRO-1)</u>              |                                   |
| Silver iodobromide emulsion (Em-5)                                 | 0.3                               |
| UV Absorber (UV-1)                                                 | 0.07                              |
| UV Absorber (UV-2)                                                 | 0.1                               |
| Additive (HS-1)                                                    | 0.2                               |
| Additive (HS-2)                                                    | 0.1                               |
| High-boiling point solvent (Oil-1)                                 | 0.07                              |
| High-boiling point solvent (Oil-2)                                 | 0.07                              |
| Gelatin                                                            | 0.8                               |
| <u>Twelfth layer: Second protective layer (PRO-2)</u>              |                                   |
| Alkali-soluble matting agent<br>(average particle size, 2 $\mu$ m) | 0.13                              |
| polymethyl methacrylate<br>(average particle size, 3 $\mu$ m)      | 0.02                              |
| Gelatin                                                            | 0.5                               |

Besides the compounds mentioned above, a coating aid SU-2, a dispersion aid SU-1, a hardener H-1, a hardener H-2, as well as dyes AI-1 and AI-2 were also added, as appropriate, to the respective layers. All of the emulsions used in sample No. 401 were monodispersed emulsions with a higher AgI content in the interior than in the surface, and they had the following characteristics:

Em-1: average AgI content, 7.5 mol %; octahedral; grain size, 0.55  $\mu$ m

Em-2: average AgI content, 2.5 mol %; octahedral; grain size, 0.36  $\mu$ m

Em-3: average AgI content, 8.0 mol %; octahedral; grain size, 0.84  $\mu$ m

Em-4: average AgI content, 8.5 mol %; octahedral; grain size, 1.02  $\mu$ m

Em-5: average AgI content, 2.0 mol %; octahedral; grain size, 0.08  $\mu$ m

#### Preparation of sample Nos. 402-415

Sample Nos. 402-415 were prepared by repeating the procedure of preparing of preparing sample No. 401 except that the compounds listed in Table 4 were added to the spectral sensitizers contained in the seventh layer.

Sample Nos. 401-415 were subjected to wedge exposure in the usual manner and subsequently processed as in Example 1.

The sensitivity and raw stock stability of sample Nos. 401-415 were evaluated as in Example 1. The results are shown in Table 4, in which the sensitivity is expressed in relative values, with the value for sample No. 401 being taken as 100, and both sensitivity and raw stock stability are related to green light.

-continued

| Sample No. | Compound   | Amount (mol/mol AgX) | Sensitivity | Raw stock stability |
|------------|------------|----------------------|-------------|---------------------|
| Invention  | 405 CR-5   | $3.4 \times 10^{-5}$ | 48          | 72                  |
|            | 406 II-1   | $3.4 \times 10^{-5}$ | 149         | 78                  |
|            | 407 II-2   | $3.4 \times 10^{-5}$ | 152         | 79                  |
|            | 408 II-2   | $6.8 \times 10^{-5}$ | 156         | 76                  |
|            | 409 II-36  | $3.4 \times 10^{-5}$ | 139         | 75                  |
|            | 410 II-36  | $6.8 \times 10^{-5}$ | 141         | 74                  |
|            | 411 II-62  | $3.4 \times 10^{-5}$ | 129         | 73                  |
|            | 412 III-1  | $3.4 \times 10^{-5}$ | 132         | 74                  |
|            | 413 III-2  | $3.4 \times 10^{-5}$ | 135         | 73                  |
|            | 414 III-22 | $3.4 \times 10^{-5}$ | 128         | 73                  |
|            | 415 III-44 | $3.4 \times 10^{-5}$ | 131         | 74                  |

| Sample No. | Compound | Amount (mol/mol AgX) | Sensitivity | Raw stock stability |
|------------|----------|----------------------|-------------|---------------------|
| Comparison | 401      | —                    | 100         | 58                  |
|            | 402 CR-1 | $3.4 \times 10^{-5}$ | 85          | 64                  |
|            | 403 CR-3 | $3.4 \times 10^{-5}$ | 86          | 68                  |
|            | 404 CR-3 | $6.8 \times 10^{-5}$ | 59          | 69                  |

15 As Table 4 shows, the samples of the present invention were improved in terms of both sensitivity and raw stock stability.



-continued

Y-1



Y-2



CC-1



CM-1



D-1



5,166,046

67



68

-continued

D-2



D-3



HS-1



HS-2



H-1

[(CH2=CHSO2CH2)3CCH2SO2(CH2)2]2N(CH2)2SO3K

H-2



Su-1



Su-2



SC-1

-continued



SC-2



Oil-1



Oil-2



Oil-3



AI-1



AI-2



UV-1



UV-2

Compounds used in comparisons

CR-1



-continued

CR-2

CR-3

CR-4

CR-5

30

As demonstrated by Examples 1-4, the present invention provides a silver halide photographic material that is low in fog, that has enhanced spectral sensitivity and that can be stored for a prolonged period without deterioration after its preparation (i.e., has good raw stock 35 stability).

What is claimed is:

1. A silver halide photographic material having one or more light-sensitive silver halide emulsion layers on a support, which said photographic material is characterized in that at least one of said light-sensitive emulsion layers contains silver halide grains that are spectrally sensitized with at least one of the spectral sensitizers represented by the following general formula (Ia) or 40 (Ib) and further contains at least one of the compounds 45 represented by the following formula (II)



R<sub>1</sub> and R<sub>2</sub> are each independently a substituted or unsubstituted alkyl group; X<sub>1</sub> is a charge balancing counter ion; K<sub>1</sub> represents a value of zero or more for 65 neutralizing electric charges;

Y<sub>1</sub> and Y<sub>2</sub> are each an oxygen atom, a sulfur atom, a selenium atom, a tellurium atom or

V<sub>1</sub>-V<sub>8</sub> are each a hydrogen atom, an alkyl group, an alkoxy group, a halogen atom, a phenyl group, a hydroxyl group, a cyano group, an alkoxy carbonyl group, a carbamoyl group, a sulfamoyl group, or a sulfonyl group, provided that V<sub>1</sub> and V<sub>2</sub>, or V<sub>2</sub> and V<sub>3</sub>, or V<sub>3</sub> and V<sub>4</sub>, or V<sub>5</sub> and V<sub>6</sub>, or V<sub>6</sub> and V<sub>7</sub> or V<sub>7</sub> and V<sub>8</sub> may combine with each other to form a benzene ring, a cyclohexene ring or a thiophene ring; R<sub>4</sub> is a substituted or unsubstituted alkyl or aryl group; W<sub>1</sub>-W<sub>4</sub> are each a hydrogen atom, an alkyl group or a phenyl group, provided that W<sub>1</sub> and W<sub>2</sub> and/or W<sub>3</sub> and W<sub>4</sub> may combine with each other to form a benzene ring, a cyclohexene ring, a thiophene ring or a naphthalene group; R<sub>3</sub> is a hydrogen atom, an alkyl group, an aralkyl group, an aryl group, a heterocyclic group or an acidic nucleus containing group;



where Z<sub>3</sub> is an oxygen atom, a sulfur atom, a selenium atom, a tellurium atom or

30  
—N—R<sub>4</sub>;

group; V<sub>21</sub>, V<sub>23</sub> and V<sub>24</sub> are each a hydrogen atom, a halogen atom, an aryl group, a substituted or unsubstituted alkyl group, an alkoxy group, an

alkoxycarbonyl group, a carboxyl group, a hydroxyl group or a cyano group,  $V_{22}$  provided that  $V_{21}$  and  $V_{22}$ , or  $V_{22}$  and  $V_{23}$  or  $V_{23}$  and  $V_{24}$  may be condensed together to form a benzene ring;  $R_{21}$ ,  $R_{22}$ ,  $R_{23}$ ,  $R_{24}$  and  $R_{25}$  are each a hydrogen atom, a halogen atom, a hydroxyl group, an alkyl group, an alkoxy group, an aryl group; and  $R_{26}$  is a substituted or unsubstituted alkyl or aryl group.

2. A silver halide photographic material according to claim 1 wherein the spectral sensitizer represented by the general formula (Ia) is added in an amount of  $2 \times 10^{-6}$  to  $1 \times 10^{-2}$  mole per mole of silver halide.

3. A silver halide photographic material according to claim 1 wherein the spectral sensitizer represented by the general formula (Ia) is added in an amount of  $5 \times 10^{-6}$  to  $5 \times 10^{-3}$  moles per mole of silver halide.

4. A silver halide photographic material according to claim 1 wherein the compound represented by the general formula (II) is used in an amount of  $1 \times 10^{-8}$  to  $1 \times 10^{-2}$  mole per mole of silver halide in the emulsion.

5. A silver halide photographic material according to claim 1 wherein the molar ratio of the spectral sensitizer of the general formula (Ia) or (Ib) to the compound of the general formula (II) is within the range of 10:1 to 1:100.

6. A silver halide photographic material according to claim 1 wherein the molar ratio of the spectral sensitizer of the general formula (Ia) or (Ib) to the compound of the general formula (II) is within the range of 2:1 to 1:10.

7. A silver halide photographic material according to claim 1 wherein the spectral sensitizer of the general formula (Ia) or (Ib) is added simultaneously with the compound of the general formula (II).

8. A silver halide photographic material according to claim 1 wherein said silver halide grains have a core/-shell structure.

9. A silver halide photographic material according to claim 8 wherein the shell of said silver halide grains is further coated with another shell having a different silver halide composition to provide a multi-layered shell.

10. A silver halide photographic material according to claim 8 wherein said silver halide grains have a shell with a silver iodide content of 2-40 mol %.

11. A silver halide photographic material according to claim 8 wherein said silver halide grains have a shell with a silver iodide content of 10-40 mol %.

15. 12. A silver halide photographic material according to claim 8 wherein said silver halide grains have a shell with a silver iodide content of 15-40 mol %.

13. A silver halide photographic material according to claim 1 wherein said silver halide grains are in the form of a normal crystal, a crystal containing twins or a tabular crystal having an aspect ratio of 5 or more.

20. 14. A silver halide photographic material according to claim 13 wherein said silver halide grains are tabular grains having a size of 0.2-30  $\mu\text{m}$  in terms of the diameter of an equivalent circle.

15. 15. A silver halide photographic material according to claim 13 wherein said silver halide grains are tabular grains having a thickness of no more than 0.5  $\mu\text{m}$ .

30. 16. A silver halide photographic material according to claim 1 wherein the spectral sensitizer represented by the general formula (Ib) is added in the amount of  $2 \times 10^{-6}$  to  $1 \times 10^{-2}$  mole per mole of silver halide.

35. 17. A silver halide photographic material according to claim 1 wherein the spectral sensitizer represented by the general formula (Ib) is added in an amount of  $5 \times 10^{-6}$  to  $5 \times 10^{-3}$  moles per mole of silver halide.

\* \* \* \* \*